

## UNITED STATES PATENT OFFICE

2,647,046

## JET COMBUSTION FUEL

Jack M. Godsey, Wenonah, N. J., assignor to Socony-Vacuum Oil Company, Incorporated, a corporation of New York

No Drawing. Application May 24, 1949,  
Serial No. 95,151

9 Claims. (Cl. 52—5)

1

This invention is directed to improved fuels utilizable in jet combustion devices. It is particularly directed to jet combustion fuels having improved jet combustion properties through the addition thereto of small amounts of an additive material.

The simplest form of jet combustion mechanism is a tube with one end closed, in which a combustible is burned. The expanding gases of combustion issuing from the open end of the tube give rise to a reaction effect which drives the tube in a direction opposite to that of the emission of the gases. The most complicated forms presently proposed consist of the same propulsion or jet tube, plus a compressor to supply air for combustion, plus a gas turbine which extracts enough energy from the departing gases to drive the compressor. In present commercial forms, the compressor and turbine are assembled axially upon a common shaft, spaced far enough apart to permit a number of combustion chambers to be arranged about the shaft between the compressor and turbine with an exhaust tube extending rearwardly from the turbine. In essence, the term jet combustion, as now commonly applied, and as used in this specification, refers to a method of combustion wherein fuel is continuously introduced into and continuously burned in a confined space for the purpose of deriving power directly from the hot products of combustion.

In practice, the range of conditions over which a jet combustion device may operate may become quite limited for ill-chosen or ill-adapted fuels. Even though a combustible mixture be present, the flame will be blown out if the rate of fuel feed is too far increased. Yet, high rates of fuel feed are necessary to obtain high heat release, which is high power delivery. Fuels with low blow-out levels can furnish only limited power and limited flexibility under conditions of operation. Consequently, the flame stability of a fuel is of major importance.

It has been found that flame stability of a fuel is correlated with a property of the fuel which is readily reproducible on a laboratory basis, using apparatus which is simple when compared to a commercial combustion tube, and with considerably less procedural difficulty. This correlated property is the rate of flame propagation as measured in a Bunsen-type burner, using the method of Smith and Pickering [J. Res. Natl. Bur. Stds. 17, (1936)]. In this procedure, the rate of flame propagation is measured at a number of fuel-air ratios by photographing the flame and measuring the slope of the flame cone. Desirable levels of commercial operability may be found in fuels having rates of flame propagation of the order of 1.4 feet per second and higher.

2

Benzol, an excellent fuel, has a rate of flame propagation of about 1.6 feet per second, at a fuel mixture temperature of 230° F., a pressure of 1 atmosphere, and an air flow rate of 3.15 pounds/hour.

As is well known to those familiar with the art, in the operation of jet combustion devices, deposits of a sootlike character are formed within the combustion chamber and in subsequent portions of the apparatus. These deposits cause operating difficulties by interfering with combustion in the combustion chamber and by damaging the turbine.

The present invention is predicated upon the discovery that small amounts of thiophene tar, disclosed in U. S. Patent No. 2,450,659, or of extracts of thiophene tar obtained by solvent treatment, when added to a fuel, will materially improve the combustion stability thereof.

Further, it has been found that small amounts of thiophene tar or of extracts of thiophene tar obtained as hereinafter disclosed, when mixed with fuels used in jet combustion devices, materially reduce the soot deposits formed during combustion.

As shown in U. S. Patent No. 2,450,659 and in copending application for Letters Patent, Serial Number 721,453, filed on January 10, 1947, now U. S. Patent No. 2,515,927, issued on July 18, 1950, thiophene tar and thiophene are prepared by separately preheating sulfur and one or more normal aliphatic hydrocarbons selected from the group consisting of normal butane, normal butenes, and butadienes, to temperatures such that combining sulfur and the hydrocarbon material will give a mixture having a temperature in excess of about 450° C., mixing the preheated sulfur and the preheated hydrocarbon mixture, maintaining the temperature of the mixture at a temperature in excess of about 450° C. for a period of time of at least 0.01 second and reducing the temperature of the mixture to less than 450° C. Along with thiophene tar and thiophene, hydrogen sulfide and small amounts of carbon disulfide are also formed in the process.

It has been found in the operation of this process that the relative proportions of sulfur and hydrocarbon material in the charge may be varied over wide limits. Too much sulfur, however, results in poor efficiency in sulfur utilization per pass and favors the complete sulfurization of hydrocarbon material to carbon disulfide. Yet, too low a proportion of sulfur lowers the conversion per pass and ultimate yield by increasing the overall thermal degradation of hydrocarbon material. Generally speaking, best results are obtained using a weight ratio of sulfur to a hydrocarbon material varying between about

0.5 and about 4.0, although when butenes and butadienes constitute the bulk of the hydrocarbon charge, the lower limit of the weight ratio may be lower than 0.5. It should be observed, however, that for economical operation of the process, it is preferred not to use a hydrocarbon charge consisting predominantly of butadienes because of their tendency to polymerize under the conditions of the process.

The selectivity of the reaction involved in the process for the preparation of thiophene tars and thiophene depends primarily upon two variables; namely, the reaction temperature at which the normal aliphatic hydrocarbon or hydrocarbons are contacted with sulfur, and the reaction time or the time during which contact between the reactants is maintained at the reaction temperature.

The limits of operating temperature are fixed by the kinetics of the desired reaction and the kinetics of possible side reactions. It has been found in this connection, that the reaction temperature may vary between about 450° C. and about 760° C. and, preferably, between about 540° C. and about 650° C. when butane is the predominant hydrocarbon reactant in the charge, and between about 480° C. and about 590° C. when butenes and butadienes are the predominant hydrocarbon reactants in the charge. Below the lower limit of the temperature range (about 450° C.), the reaction is so slow as to require a large throughput of sulfur and a higher ratio of hydrocarbon recycle for a fixed amount of end product, thereby detracting from the economics of the operation. Above the upper limit of the temperature range, the secondary reaction of degradation of hydrocarbon material in the charge takes precedence, thereby decreasing the yield of desired product. In addition to this, high temperatures favor the formation of carbon disulfide. It must be noted, also, that at these high temperatures corrosion problems are at a maximum, corrosion increasing perceptibly with increasing temperature.

It has also been found, in connection with this process, that the optimum reaction time depends upon the temperature employed. In general, other variables remaining constant, the lower the temperature, the longer the reaction time. The reaction or contact time and the reaction temperature are somewhat fixed, one in relation to the other, by the degree of degradation of the hydrocarbon material in the charge and by the effect of formation of undesirable products which may be tolerated. Thus, too long a contact time at high temperature results in severe cracking of the hydrocarbon material in the charge. The reaction proceeds with extreme speed, the only apparent limitation being the rapidity with which heat can be supplied to the reaction mixture. The reaction is highly endothermic, requiring by experimental measure approximately 28,000 calories per gram molecular weight of thiophene produced from normal butane. The lower limit of the range of reaction time is fixed, therefore, by the engineering problem of heat transfer and by mechanical limitations such as allowable pressure drop across the reactor. Relatively long reaction times at temperatures in the neighborhood of the lower limit of the temperature range result in insufficient reaction. Accordingly, it has been found that for best results the time of reaction is fixed by the reaction temperature.

In view of the foregoing, the criteria to be

used in determining optimum operating temperatures within the range of 450° C. to 760° C. depend on the degree of conversion desired commensurate with operating costs, such as heat input and equipment cost, bearing in mind that within limits, the shorter the reaction time, and accordingly the higher the temperature, the larger the amount of end product which can be realized from a unit of given size per day.

While the relationship between the temperature of reaction and reaction time is not peculiar to the present process, it has been found that thiophene tar and thiophene may be produced by reacting sulfur and the aforesaid 4-carbon hydrocarbons at a temperature between about 450° C. and about 760° C. for a period of time selected to minimize the yields of secondary reaction products such as carbon disulfide, coke-like materials and the like at the selected temperature. Under such conditions, when operating continuously with a reactor coil of suitable size and at a practical charge rate, it has been found that the lowest practical limit of the time of reaction is of the order of 0.01 second at about 760° C. The upper practical limit of the reaction time, other variables remaining constant, will correspond to the lower limit of the reaction temperature and may be of the order of several seconds.

Separate preheating of the hydrocarbon reactant and sulfur and quenching of the reaction mixture are necessary for achieving the somewhat close control of the reaction time at a given reaction temperature. This is very important in producing the specific reaction products, thiophene and thiophene tar. It is suspected that a number of reactions occur upon contacting the hydrocarbon reactant with sulfur. In this connection, the following should be noted: cracking of the hydrocarbon reactant destroying the 4-carbon atom chain structure (said 4-carbon atom chain structure being a prerequisite for the formation of thiophene), formation of thiophene tars high in sulfur and formation of carbon disulfide. These reactions compete with one another. It has been found that the rates of the formation of lighter hydrocarbons and of the formation of carbon disulfide are somewhat slower than those required for the formation of thiophene and thiophene tar. Accordingly, proper control of the reaction time at a given reaction temperature, achieved by separate preheating, mixing, heating at a given temperature for a corresponding period of time, and quenching is necessary to produce high yields of thiophene and thiophene tar with limited yields of carbon disulfide, coke-like materials, and fixed gases, due to limited decomposition of the hydrocarbon product. The rate of the reaction producing thiophene tar is fairly close to that required for the formation of thiophene, and the yields of thiophene tar and of thiophene are approximately the same. Upon standing, the thiophene tar separates from the other products and a separation can be made by decantation or other suitable separating means.

In this process the reaction is effected preferably at atmospheric pressure or under sufficient pressure to cause the flow of the reactants through the reactor and auxiliary system under the desired reaction conditions. Tests have shown that the conversion per pass and ultimate yield of thiophene decreases with increasing pressure. However, even at appreciable pressures, thiophene and thiophene tar are, nevertheless, produced in substantial amounts.

The following example will serve as an illustration:

*Example*

A mixture containing 30 per cent by volume of 1,3-butadiene and 70 per cent by volume of normal butane was charged into a preheater at a rate of 35 grams per minute and heated to a temperature of 590° C. Sulfur was charged to a separate preheater at a rate of 28 grams per minute and heated to a temperature of 590° C. The two streams were sent through a mixing nozzle and then through a baffled tube reactor constructed of 27 per cent chromium stainless steel, maintained at a temperature of 650° C. The reaction product was quenched with a water spray passed through a small Cottrell precipitator to remove tar mist and scrubbed through a hot countercurrent caustic tower. Liquid product was condensed and separated in a water cooler and ice trap and the residual gas was metered. Of the hydrocarbon material charged, 49 per cent was converted to a liquid product and tar in approximately equal portions. The tar was separated from the liquid product by decantation.

In the practice of the present invention, the amount of thiophene tar or of thiophene tar extract employed is that which is sufficient to improve the flame stability of the fuel. For example, in the case of thiophene tar, the amount used falls within the range varying between about 0.1 per cent and 2.0 per cent by weight. The thiophene tar has limited solubility in certain base fuels, being less than 2.0 per cent in some cases. Its solubility will, of course, differ in fuels of different characteristics. The extracts of thiophene tar, on the other hand, being completely soluble in all jet combustion fuels, do not present this difficulty thereby permitting the use of a larger percentage of additive material than may be possible with the thiophene tar. The extracts of thiophene tar are usually added to the base fuel in amounts between about 0.1 per cent and about 2.0 per cent by weight. Greater amounts, up to 10 per cent, may be used if desired, although, in general, no outstanding results seem to occur. Conceivably and within the scope of the present invention, these additives may be added to jet fuels to be marketed or procured as concentrates, viz., jet combustion fuels containing upwards of 10 per cent and up to 49 per cent by weight of the additive. These concentrates are subsequently added to a jet combustion fuel in such proportions as to produce the effective concentration of additive in the fuel desired, i. e., a sufficient amount to improve the jet combustion properties of the jet combustion fuel.

The thiophene tar extracts are obtained by treating the thiophene tar with a C<sub>3</sub>-C<sub>10</sub> alkane hydrocarbon or mixtures of C<sub>3</sub>-C<sub>10</sub> alkane hydrocarbons. Typical of these C<sub>3</sub>-C<sub>10</sub> alkane hydrocarbons, are propane, isobutane, 1,3-dimethyl pentane, n-hexane, 2,3-ethyl-methyl hexane, and n-decane. The preferred solvents are C<sub>5</sub>-C<sub>8</sub> alkane hydrocarbons. In the preparation of these extracts, the thiophene tar is contacted with the hydrocarbon solvent in a suitable apparatus for the production of extracts, at temperatures varying between about 10° C. and up to about 40° C., and for a period of time sufficient to extract at least about 5 per cent by weight of the thiophene tar. There appears to be nothing critical about the relative amounts of thiophene tar and of hydrocarbon solvent to be employed.

Ordinarily, a proportion of at least about 1:1 and up to 4:1, by volume, of solvent to thiophene tar is used in one or more stages (up to four stages). The extract thus obtained is then subjected to a distillation to strip out the solvent.

For example, thiophene tar is partially soluble in such hydrocarbons as normal heptane and iso-octane (2,2,4-trimethyl-pentane). Accordingly, the thiophene tar is contacted with two parts by volume of normal heptane or iso-octane at a temperature of 25° C. for about 40 minutes, and the liquid extract phase removed and subjected to distillation to remove the normal heptane or iso-octane. The resultant product is wholly soluble in fuels of boiling ranges suitable for the usual jet combustion devices.

The jet combustion fuels of the present invention may contain other materials or additives for improving other characteristics thereof. Gum inhibitors and starting aids are mentioned by way of non-limiting examples of other additives which may be present in the jet combustion fuels of the present invention.

The addition of thiophene tar and of its extracts may be made to fuels of a fairly wide variety of boiling ranges, specific gravity, etc. Suitable base fuels for use in accordance with this invention include those having the character of light gasolines up to those having the character of gas oils: Synthetic fuels, such as those manufactured by the Fischer-Tropsch process, can be used, as can be fuels derived from coal or wood distillation. It is also contemplated to add these combustion improving additives to liquid alcohols or combinations of alcohols with other base fuels. The preferred fuel is, however, a hydrocarbon distillate fuel boiling within the range of about 100° F. to about 600° F.

The physical characteristics of typical suitable base fuels are given hereinafter for illustrative purposes:

1. Hydrocarbon distillate fuel:

|                |                              |
|----------------|------------------------------|
| Boiling range  | 105-535° F.                  |
| Gravity        | 53° A. P. I.                 |
| Vapor pressure | 5.4 Reid, pounds.            |
| Freezing point | Below -76° F.                |
| Sulfur         | 0.03%, by weight.            |
| Bromine No     | 15.                          |
| Aromatics      | 15%, by volume.              |
| Viscosity      | .773 centistokes, at 100° F. |

2. Reference fuel A:

|                |                              |
|----------------|------------------------------|
| Boiling range  | 205-225° F.                  |
| Gravity        | 71.6° A. P. I.               |
| Vapor pressure | 1.7 Reid, pounds.            |
| Freezing point | Below -76° F.                |
| Sulfur         | Nil.                         |
| Bromine No     | 0.                           |
| Aromatics      | 0.                           |
| Viscosity      | .623 centistokes, at 100° F. |

3. Reference fuel B:

|                |                              |
|----------------|------------------------------|
| Boiling range  | 320-470° F.                  |
| Gravity        | 36.5° A. P. I.               |
| Freezing point | Below -76° F.                |
| Sulfur         | 0.035%, by weight.           |
| Bromine No     | 1.                           |
| Aromatics      | 12.1%, by volume.            |
| Viscosity      | 1.48 centistokes, at 100° F. |

The following examples are given for the purpose of illustrating the present invention and for indicating the advantages thereof. It must be clearly understood, however, that these exam-

ples are non-limiting. It will be appreciated by those skilled in the art that numerous types of jet combustion fuels, other than the reference fuels described hereinbefore, may be used for the purpose contemplated herein.

Thiophene tar in a concentration of about 0.5 per cent by weight in reference fuel B was subjected to comparison test runs against the same fuel in a General Electric I-16 combustion chamber. Fuel flow and air flow were adjusted to simulate combustion conditions under actual operation in jet propelled aircraft equipped with a General Electric I-16 burner. Deposit formation was quantitatively evaluated by weighing the liners of the combustion chamber before and after burning a specified amount of fuel. The results of this test are shown in Table I.

Table I

| Fuel                                              | Deposit Weight | Reduction in Deposits |
|---------------------------------------------------|----------------|-----------------------|
|                                                   | Grams          | Percent               |
| Reference Fuel B                                  | 11.0           |                       |
| 99.5% of Reference Fuel B with 0.5% Thiophene Tar | 4.9            | 56                    |

As another example illustrative of this invention, the rate of flame propagation using reference fuel A (substantially 2,2,4-trimethylpentane) was compared with that of a blend of the reference fuel A with 0.5 per cent by weight of the n-heptane extract of thiophene tar, in accordance with the procedure of Smith and Pickering hereinbefore disclosed. The fuel mixture was maintained at a temperature of about 230° F., under a pressure of 1 atmosphere, and the air flow rate was controlled at 3.15 pounds/hour. A similar test was conducted using a blend of 99.5 per cent of reference fuel A with 0.5 per cent of the isoctane extract of thiophene tar, previously disclosed. The results of these tests are shown in Table II.

Table II

| Fuel                                                                | Rate of Flame Propagation Ft./Sec. |
|---------------------------------------------------------------------|------------------------------------|
| 100% Reference Fuel A                                               | 1.45                               |
| 99.5% Reference Fuel A with 0.5% n-heptane extract of thiophene tar | 1.60                               |
| 99.5% Reference Fuel A with 0.5% isoctane extract of thiophene tar  | 1.50                               |

It will be seen that by adding as little as 0.5 per cent of the extract material obtained from thiophene tar to the fuel, a substantial increase in rate of flame propagation is obtained, which, as indicated hereinbefore, means a substantial improvement in combustion stability.

This application is a continuation-in-part of copending application, Serial No. 744,023, filed April 25, 1947, now abandoned.

What is claimed is:

1. A liquid fuel capable of being utilized in jet-combustion mechanisms, which comprises a hydrocarbon distillate having an initial boiling point of about 40° C. and a final boiling point of about 315° C. and boiling substantially continuously between said points, and between about 0.1 per cent by weight and about 2.0 per cent by weight of thiophene tar obtained by the process which includes separately preheating sulfur and a C<sub>4</sub>-hydrocarbon selected from the group consisting of normal butane, normal butenes and

butadienes, to temperature such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; and separating the thiophene tar from said mixture.

2. A liquid fuel capable of being utilized in jet-combustion mechanisms, which comprises a hydrocarbon distillate having an initial boiling point of about 40° C. and a final boiling point of about 315° C. and boiling substantially continuously between said points, and between about 0.1 per cent by weight and about 10.0 per cent by weight of thiophene tar obtained by the process which includes separately preheating sulfur a C<sub>4</sub>-hydrocarbon selected from the group consisting of normal butane, normal butenes and butadienes, to temperatures such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; and separating the thiophene tar from said mixture.

3. A liquid fuel capable of being utilized in jet-combustion mechanisms, which comprises a hydrocarbon distillate having an initial boiling point of about 40° C. and a final boiling point of about 315° C. and boiling substantially continuously between said points, and between about 0.1 per cent by weight and about 2.0 per cent by weight of an extract of thiophene tar obtained by the process which includes separately preheating sulfur a C<sub>4</sub>-hydrocarbon selected from the group consisting of normal butane, normal butenes and butadienes, to temperatures such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; separating the

thiophene tar from said mixture; treating said thiophene tar with a C<sub>5</sub>-C<sub>8</sub> alkane hydrocarbon solvent, to produce a hydrocarbon extract; separating the hydrocarbon extract; and removing the hydrocarbon from the hydrocarbon extract, to obtain the extract.

4. A liquid fuel capable of being utilized in jet-combustion mechanisms, which comprises a hydrocarbon distillate having an initial boiling point of about 40° C. and a final boiling point of about 315° C. and boiling substantially continuously between said points, and between about 0.1 per cent by weight and about 10.0 per cent by weight of an extract of thiophene tar obtained by the process which includes separately preheating sulfur a C<sub>4</sub>-hydrocarbon selected from the group consisting of normal butane, normal butenes and butadienes, to temperatures such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; separating the thiophene tar from said mixture; treating said thiophene tar with a C<sub>5</sub>-C<sub>8</sub> alkane hydrocarbon solvent, to produce a hydrocarbon extract; separating the hydrocarbon extract; and removing the hydrocarbon from the hydrocarbon extract, to obtain the extract.

5. A liquid fuel capable of being utilized in jet-combustion mechanisms, which comprises a hydrocarbon distillate having an initial boiling point of about 40° C. and a final boiling point of about 315° C. and boiling substantially continuously between said points, and between about 0.1 per cent by weight and about 2.0 per cent by weight of an extract of thiophene tar obtained by the process which includes separately preheating sulfur a C<sub>4</sub>-hydrocarbon selected from the group consisting of normal butane, normal butenes and butadienes, to temperatures such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; separating the thiophene tar from said mixture; treating said thiophene tar with a C<sub>3</sub>-C<sub>10</sub> alkane hydrocarbon solvent, to produce a hydrocarbon extract; separating the hydrocarbon extract; and removing the hydrocarbon from the hydrocarbon extract, to obtain the extract.

6. A liquid fuel capable of being utilized in jet-combustion mechanisms, which comprises a hydrocarbon distillate having an initial boiling point of about 40° C. and a final boiling point of about 315° C. and boiling substantially continuously between said points, and between about 0.1 per cent by weight and about 2.0 per cent by weight of an extract of thiophene tar obtained by the process which includes separately pre-

point of about 40° C. and a final boiling point of about 315° C. and boiling substantially continuously between said points, and between about 0.1 per cent by weight and about 10.0 per cent by weight of an extract of thiophene tar obtained by the process which includes separately preheating sulfur a C<sub>4</sub>-hydrocarbon selected from the group consisting of normal butane, normal butenes, and butadienes, to temperatures such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; separating the thiophene tar from said mixture; treating said thiophene tar with a C<sub>3</sub>-C<sub>10</sub> alkane hydrocarbon solvent, to produce a hydrocarbon extract; separating the hydrocarbon extract; and removing the hydrocarbon from the hydrocarbon extract, to obtain the extract.

7. A liquid fuel capable of being utilized in jet-combustion mechanisms, which comprises a hydrocarbon distillate having an initial boiling point of about 40° C. and a final boiling point of about 315° C. and boiling substantially continuously between said points, and between about 0.1 per cent by weight and about 2.0 per cent by weight of an extract of thiophene tar obtained by the process which includes separately preheating sulfur a C<sub>4</sub>-hydrocarbon selected from the group consisting of normal butane, normal butenes and butadienes, to temperatures such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; separating the thiophene tar from said mixture; treating said thiophene tar with normal heptane, to produce a hydrocarbon extract; separating the hydrocarbon extract; and removing the normal heptane from the hydrocarbon extract, to obtain the extract.

8. A liquid fuel capable of being utilized in jet-combustion mechanisms, which comprises a hydrocarbon distillate having an initial boiling point of about 40° C. and a final boiling point of about 315° C. and boiling substantially continuously between said points, and between about 0.1 per cent by weight and about 2.0 per cent by weight of an extract of thiophene tar obtained by the process which includes separately pre-

## 11

heating sulfur a C<sub>4</sub>-hydrocarbon selected from the group consisting of normal butane, normal butenes and butadienes, to temperatures such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; separating the tar from said mixture; treating said thiophene tar with isooctane, to produce a hydrocarbon extract; separating the hydrocarbon extract; and removing the isooctane from the hydrocarbon extract, to obtain the extract.

9. A liquid fuel capable of being utilized in jet-combustion mechanisms, which comprises a hydrocarbon distillate having an initial boiling point of about 40° C. and a final boiling point of about 315° C. and boiling substantially continuously between said points, and a minor proportion, sufficient to improve the combustion properties thereof, of a material selected from the groups consisting of (1) thiophene tar obtained by the process which includes separately pre-

5

10

15

20

25

30

35

## 12

heating sulfur a C<sub>4</sub>-hydrocarbon selected from the group consisting of normal butane, normal butenes and butadienes, to temperatures such that combining said sulfur and said C<sub>4</sub>-hydrocarbon will give a reaction mixture having a temperature falling within the range varying between about 450° C. and about 760° C.; mixing the preheated sulfur and the preheated C<sub>4</sub>-hydrocarbon; reacting said preheated sulfur with said preheated C<sub>4</sub>-hydrocarbon at a reaction temperature falling within the range varying between about 450° C. and about 760° C. for a period of time selected to minimize the yields of hydrocarbons containing less than four carbon atoms per molecule and carbon disulfide at said reaction temperature, to yield a mixture containing thiophene tar; immediately reducing the temperature of the mixture containing said thiophene tar to a temperature of less than about 450° C.; and separating the thiophene tar from said mixture; and (2) an extract of said thiophene tar obtained by treating said thiophene tar with a C<sub>3</sub>-C<sub>10</sub> alkane hydrocarbon solvent, to produce a hydrocarbon extract; separating the hydrocarbon extract; and removing the hydrocarbon from the hydrocarbon extract, to obtain the extract.

JACK M. GODSEY.

References Cited in the file of this patent  
UNITED STATES PATENTS

| Number    | Name        | Date          |
|-----------|-------------|---------------|
| 2,450,659 | Hansford    | Oct. 5, 1948  |
| 2,515,927 | Lukasiewicz | July 18, 1950 |